

# United States Patent Office

3,472,713

1

3,472,713

3,472,715

**FUSIBLE AROMATIC NITROCOMPOUND EXPLOSIVE COMPOSITION CONTAINING PARTICULAR WAX AS A DESENSITIZER**

Adolf Berthmann and Paul Lingens, Leverkusen, Germany, assignors to Dynamit Nobel Aktiengesellschaft, a corporation of Germany.

a corporation of Germany  
No Drawing. Filed July 17, 1968, Ser. No. 745,357  
Claims priority, application Germany, July 20, 1967,

Priority, application Germany, July  
D 53,636  
Int. Cl. C06b 9/04, 15/02, 3/00

## 11 Claims

#### ABSTRACT OF THE DISCLOSURE

Explosive compositions on a basis of fusible aromatic nitrocompounds and nitramines and/or nitric esters having incorporated therein as desensitizer a wax of a mixture of polychloronaphthalenes obtained in the chlorination and refining of naphthalene.

This invention relates to the use of soluble desensitizers for the desensitization of castable explosives prepared on a basis of aromatic nitrocompounds and nitramines and/or nitric esters.

More particularly this invention relates to the use of waxes comprising a mixture of polychloronaphthalenes obtained in the chlorination and refining of naphthalene, for the desensitization of castable explosives prepared on a basis of aromatic nitro compounds and nitramines and/or nitric esters and/or powdered metals and/or known desensitizers.

The aforesaid waxes are soluble in aromatic nitro compounds and are known under the commercial name "Nibrenwaches." (Literature source: Ullmanns Encyclopädie der Technischen Chemie, publishing house Urban & Schwarzenberg, Munich-Berlin, 1954, vol. 5, page 474.) "Nibrenwachs" here is a mixture of polychloronaphthalenes. The production of these mixtures of isomeric polychloronaphthalenes is mentioned, for example, in the U.S. Patent 1,111,289 and in the German Patent 548,260 (compare Ullmann, page 474).

part Ummann, page 474). It is known that castable explosives prepared on a basis of aromatic nitro compounds and nitramines and/or nitric esters can be desensitized by the addition of waxes thereto; for example, 1% wax is often added to Composition B (60 parts hexogen, 40 parts trinitrotoluene) and also to the Pentolite mixture (50 parts pentaerythritol tetranitrate and 50 parts trinitrotoluene). The latter wax is not soluble in molten TNT. In order to form a stable emulsion of the explosive and wax, emulsifying aids are often added, as for example, lecithin as an emulsifier and nitrocellulose as a stabilizer.

In addition, waxes and the necessary accompanying emulsifying aids are frequently added to metalcontaining explosive mixtures, such as, for example, a mixture of

|                 | Percent |
|-----------------|---------|
| Trinitrotoluene | 28.9    |
| Hexogen         | 31.2    |
| Aluminium       | 35.1    |
| Paraffin wax    | 4.0     |
| Lecithin        | 0.2     |
| Nitrocellulose  | 0.6     |

The use of such waxes and the accompanying emulsifying aids, however, is associated with disadvantages. Since wax, lecithin and nitrocellulose are natural substances or derivatives of natural substances, their characteristics can-

2

not always be precisely controlled and accordingly the formation of a stable emulsion is not always assured. Furthermore, the waxes used hitherto were characterized by a low density, so that the resultant density of the entire explosive mixture was lowered.

5 the explosive mixture was lowered.  
These disadvantages can be eliminated by employing  
as desensitizer soluble waxes, that is waxes soluble in the  
explosive mixture. The solubility of the desensitizer waxes  
make it possible to proceed without resorting to an emul-  
10 sion, the latter being often quite difficult to prepare. Fur-  
thermore, the aforesaid soluble waxes having high den-  
sities and namely densities in the range of 1.5 to 1.7 g./  
cm.<sup>3</sup>.

15 It is most surprising that, in comparison to the other waxes, and namely the insoluble waxes, a better desensitization to rapid heating is achieved by the use of the soluble waxes, while desensitization to shock and impact is substantially equal to that realized with the waxes used hitherto.

20 The desensitizing effect of the wax additives, in accordance with the invention as compared to the insoluble waxes, was measured in the following manner: 0.4 g. of an explosive mixture without wax or with an insoluble or soluble wax was placed in a glass reaction vessel either in the form of a single piece or in a finely ground state. The glass vessel was then immersed in a molten bath of Wood's metal. The molten metal bath was then adjusted to a constant predetermined temperature. The time it took to produce flashing or explosion of the mixture was then determined. The longer the period of time, 25 the more tolerant the explosive mixture is of thermal stresses.

As illustrative embodiments of a manner in which the invention may be practised, the following examples are presented.

In Examples 1 to 4, the explosive mixtures were pulverized, while the explosive mixtures of Examples 5, 6 and 7 were used in pieces having a weight of 0.4 g.

40 The terms TNT, hexogen and tetryl as used heretofore and in the examples, designate respectively trinitrotoluene, cyclotrimethylenetrinitramine, and 2,4,6 - trinitrophenyl-methylnitramine.

### EXAMPLE 1

The time required to produce flashing or explosion of TNT with and without desensitizers, was measured at 340° C. The following data were obtained:

|    |                                                                                                                                                                         | Seconds |
|----|-------------------------------------------------------------------------------------------------------------------------------------------------------------------------|---------|
| 50 | 100 parts TNT                                                                                                                                                           | 74      |
|    | 30 parts TNT, 5 parts "Nierenwachs" D 116 (softening point: 113° C.; dropping point: 116° C.; specific density: 1.66 g./cm. <sup>3</sup> ; content of chlorine: 52-54%) | 82      |
| 55 | 30 parts TNT, 5 parts "Nierenwachs" D 130 (softening point: 130° C.; dropping point: 132° C.; specific density: 1.73 g./cm. <sup>3</sup> ; content of chlorine: 57-59%) | 82      |
| 60 | 30 parts TNT, 5 parts Montan wax                                                                                                                                        | 35      |

The above example clearly establishes that "Nibrenwachs," when used according to the invention, acts as a better desensitizer than Montan wax. Montan wax, although it is a desensitizer against shock and impact, acted to reduce the time considerably for explosion to occur.

**EXAMPLE 2**

70 In the case of explosive mixtures of TNT and aluminum powder, the following times were measured at 340° C. for flashing or explosion to take place.

|                                                                                                 | Seconds |
|-------------------------------------------------------------------------------------------------|---------|
| 30 parts TNT, 35 parts powdered aluminum                                                        | 59      |
| 30 parts TNT, 33 parts powdered aluminum, 5 parts ceresin wax                                   | 26      |
| 30 parts TNT, 33 parts powdered aluminum, 5 parts Nibrenwachs D 116 N (softening point 116° C.) | 65      |

This example, too, clearly demonstrates an improvement in the desensitizing action when Nibrenwachs is used.

#### EXAMPLE 3

Explosive mixtures corresponding to Composition B were measured at 238° C. for the time required to produce flashing or explosion:

|                                                          | Seconds |
|----------------------------------------------------------|---------|
| 39 parts TNT, 60 parts hexogen                           | 33      |
| 39 parts TNT, 60 parts hexogen, 1 part Montan wax        | 32      |
| 39 parts TNT, 60 parts hexogen, 1 part Nibrenwachs D 116 | 47      |

The desensitizing action of the Nibrenwachs against thermal stresses in explosives of the Composition B type is readily apparent. The Montan wax content was increased to 5 parts and the mixture again tested. However, the time of 32 seconds would not be improved on at this temperature.

#### EXAMPLE 4

In the case of explosive mixtures of TNT, hexogen and powdered aluminum, the following times were measured at 235° C. for producing flashing or explosion. In addition, the following specific weights were determined:

|                                                                                                                                                                           | Time<br>(seconds) | Spec. Wt.<br>(g./cm. <sup>3</sup> ) | 35 |
|---------------------------------------------------------------------------------------------------------------------------------------------------------------------------|-------------------|-------------------------------------|----|
| 35 parts TNT, 40 parts hexogen, 25 parts powdered aluminum                                                                                                                | 30                | 1.85                                |    |
| 30 parts TNT, 40 parts hexogen, 25 parts powdered aluminum, 5 parts desensitizer, consisting of: 4.2 parts paraffin wax, 0.7 parts nitrocellulose, 0.1 part part lecithin | 29                | 1.77                                | 40 |
| 30 parts TNT, 40 parts hexogen, 25 parts powdered aluminum, 5 parts Nibrenwachs D 130                                                                                     | 37                | 1.88                                |    |
| 30 parts TNT, 40 parts hexogen, 25 parts powdered aluminum, 4.5 parts Nibrenwachs D 130, 0.8 parts paraffin wax                                                           | 36                | 1.86                                | 45 |

The desensitizing action and the improvement in density brought about by the addition of Nibrenwachs are clearly apparent in this example. The simultaneous use of soluble Nibrenwachs and of emulsion-forming paraffin wax improves the casting properties somewhat, without, however, reducing safety from thermal stress.

#### EXAMPLE 5

The following times were determined for explosive mixtures of tetryl and TNT (tetrytol) at 230° C. for producing flashing or explosion:

|                                                         | Seconds |
|---------------------------------------------------------|---------|
| 70 parts tetryl, 30 parts TNT                           | 28      |
| 69 parts tetryl, 30 parts TNT, 1 part Montan wax        | 32      |
| 69 parts tetryl, 30 parts TNT, 1 part Nibrenwachs D 116 | 43      |

#### EXAMPLE 6

In the case of explosive mixtures of TNT and nitropentaerythrite [=PETN], the following times were determined at 230° C. for producing flashing or explosion:

|                                                                                                                     | Seconds |
|---------------------------------------------------------------------------------------------------------------------|---------|
| 50 parts TNT, 50 parts nitropentaerythrite                                                                          | 27      |
| 50 parts TNT, 49 parts nitropentaerythrite, 0.84 parts paraffin wax, 0.14 parts nitrocellulose, 0.02 parts lecithin | 31      |
| 50 parts TNT, 49 parts nitropentaerythrite, 1 part Nibrenwachs D 116                                                | 35      |

#### EXAMPLE 7

Explosive mixtures of tetryl, trinitrobenzene and hexogen were prepared and evaluated for the time required at 230° C. to produce flashing or explosion. The following data were obtained:

|                                                                                       | Seconds |
|---------------------------------------------------------------------------------------|---------|
| 16 parts tetryl, 24 parts trinitrobenzene, 60 parts hexogen                           | 45      |
| 16 parts tetryl, 24 parts trinitrobenzene, 59 parts hexogen, 1 part Montan wax        | 44      |
| 16 parts tetryl, 24 parts trinitrobenzene, 59 parts hexogen, 1 part Nibrenwachs D 130 | 55      |

The improvement in the desensitization produced by the use of Nibrenwachs in accordance with the invention is readily apparent from Examples 5 to 7.

We claim:

1. An explosive composition comprising a fusible aromatic nitro compound selected from the group consisting of trinitrotoluene, 2,4,6 - trinitrophenylmethylnitramine, and trinitrobenzene and a wax as desensitizer consisting of a mixture of polychloronaphthalenes obtained in the chlorination and refinement of naphthalene.
2. An explosive composition according to claim 1 additionally containing at least one member selected from the group consisting of nitramines, nitric esters and powdered metals.
3. An explosive composition according to claim 1 comprising 30 parts trinitrotoluene and 5 parts of a wax consisting of a mixture of polychloronaphthalenes obtained in the chlorination and refinement of naphthalene, having a softening point of 130° C.
4. An explosive composition according to claim 1 comprising 30 parts trinitrotoluene, 33 parts powdered aluminum and 5 parts of a wax consisting of a mixture of polychloronaphthalenes obtained in the chlorination and refinement of naphthalene, having a softening point of 116° C.
5. An explosive composition according to claim 1 comprising 39 parts trinitrotoluene, 60 parts cyclotrimethyl-enertrinitramine, and 1 part of a wax consisting of a mixture of polychloronaphthalenes obtained in the chlorination and refinement of naphthalene, having a softening point of 116° C.
6. An explosive composition according to claim 1 comprising 30 parts trinitrotoluene, 40 parts cyclotrimethyl-enertrinitramine, 25 parts powdered aluminum, and 5 parts of a wax consisting of a mixture of polychloronaphthalenes obtained in the chlorination and refinement of naphthalene, having a softening point of 130° C.
7. An explosive composition according to claim 1 comprising 69 parts, 2,4,6 - trinitrophenylmethylnitramine, 30 parts trinitrotoluene and 1 part of a wax consisting of a mixture of polychloronaphthalenes obtained in the chlorination and refinement of naphthalene, having a softening point of 130° C.
8. An explosive composition according to claim 1 comprising 50 parts trinitrotoluene, 49 parts pentaerythritol tetranitrate, and 1 part of a wax consisting of a mixture of polychloronaphthalenes obtained in the chlorination and refinement of naphthalene, having a softening point of 116° C.
9. An explosive composition according to claim 1 comprising 16 parts tetryl, 2,4,6 - trinitrophenylmethylnitramine, 24 parts trinitrobenzene, 59 parts cyclotrimethyl-enertrinitramine, and 1 part of a wax consisting of a mixture of polychloronaphthalenes obtained in the chlorination and refinement of naphthalene, having a softening point of 130° C.
10. An explosive composition according to claim 1, wherein said wax is present in a ratio of 1 part wax: 5

to 100 parts explosive components comprising a fusible aromatic nitro compound and mixtures thereof with at least one member of the group of nitramines, nitric esters and powdered metals.

11. A method of desensitizing explosive compositions comprising fusible aromatic nitro compounds selected from the group consisting of trinitrotoluene, 2,4,6-trinitrophenylmethylnitramine, and trinitrobenzene comprising incorporating into said composition a wax consisting of a mixture of polychloronaphthalenes obtained in the chlorination and refinement of naphthalene.

## References Cited

## UNITED STATES PATENTS

2,982,641 5/1961 Dawson et al. \_\_\_\_ 149—105 X  
3,000,720 9/1961 Baer et al. \_\_\_\_ 149—105 X

5 C. D. QUARFORTH, Primary Examiner  
S. J. LECHERT, Assistant Examiner.

U.S. CL. X.R.

10 171—93, 94; 149—105, 106, 107

UNITED STATES PATENT OFFICE  
CERTIFICATE OF CORRECTION

Patent No. 3,472,713 Dated Oct. 14, 1969

Inventor(s) ADOLF BERTHMANN and PAUL LINGENS

It is certified that error appears in the above-identified patent and that said Letters Patent are hereby corrected as shown below:

Column 1, line 29, cancel the period after "naphthalene" and insert a comma; column 1, lines 35-36, "Nibrenwaches." should be --Nibrenwachse.--; column 1, line 47, "exacle" should be --example--.

SIGNED AND  
SEALED  
**JUL 7 1970**

**(SEAL)**

Attest:

Edward M. Fletcher, Jr.

Attesting Officer

WILLIAM E. SCHUYLER, JR.  
Commissioner of Patents